

## UNITED STATES PATENT OFFICE

2,507,180

## CYANO ACETAMINO COLOR COUPLERS

Ilmari F. Salminen and Arnold Weissberger,  
Rochester, N. Y., assignors to Eastman Kodak  
Company, Rochester, N. Y., a corporation of  
New Jersey

No Drawing. Application February 8, 1947,  
Serial No. 727,298

9 Claims. (Cl. 95—6)

1

This invention relates to photography and particularly to compounds which form dyes by coupling with the developing agent to produce colored images.

It is known that colored photographic images may be formed by using a developer which produces a colored compound on development. The colored compound thus formed is deposited adjacent the silver grains of the silver image during the developing. It is also known that a colored image may be formed by adding to certain developer solutions or by incorporating in the silver halide emulsion before or after exposure a compound which couples during development with the oxidation product of the developing agent and forms a colored compound which is likewise deposited adjacent the silver grains of the silver image during development. Such a compound which is employed in conjunction with a developing agent for the silver and which couples with the oxidation product of the developing agent during development is referred to herein as a coupling compound or coupler.

The present invention concerns new or improved color-forming developers comprising primary aromatic amino developing agent and a coupler as hereinafter defined and also includes a new or improved color development process which consists in developing a reducible silver salt image in a photographic element with the aid of a primary aromatic amino developer and in the presence of a coupler as hereinafter defined. It also includes photographic sensitive elements having such coupler in one or more emulsion layers.

We have found that compounds of the following structure are valuable couplers for color photography and produce blue to purple, gray to blue-green and gray to purple images on color development:



where R is an aromatic nucleus or aromatic system and the position in the aromatic nucleus para or ortho to the hydroxyl group is unsubstituted with an irreplaceable group, that is, is unsubstituted or is substituted with a replaceable group such as chlorine.

The compounds of our invention are prepared by treating an aminophenol or aminonaphthol with ethyl cyano acetate, or with ethyl acetate or another suitable solvent, and cyano acetyl azide. Other substituent groups such as chlorine, bromine, methyl, ethyl, methoxy, ethoxy, etc., may be present in the aromatic nucleus as long as the position in the aromatic nucleus para to the hydroxyl group is unsubstituted or is substituted

with a group which is replaceable in the coupling reaction.

Suitable amino phenols or amino naphthols which may be used in the preparation of our 5 couplers are o-aminophenol, m-aminophenol, p-chloro-o-aminophenol, 2-amino-5-chlorophenol, 5-amino-1-naphthol, 4-chloro-5-amino-1-naphthol and 2-amino-1-naphthol.

The compounds 2-cyanoacetaminophenol and 10 5-cyanoacetamino-1-naphthol illustrate couplers which may be used according to our invention. These couplers may be produced as follows:

## 2-CYANOACETAMINO PHENOL

## Method 1

A mixture of 30 cc. of ethyl cyanoacetate and 10.9 g. of o-amino phenol was heated to a boil in a distilling flask. At about 190° C. alcohol was formed and collected. Heating was continued until the temperature of the distillate vapors had risen to 180°, the theoretical amount of alcohol being collected. A solid, which crystallized from the distillate on cooling was filtered and washed on the filter with 50 cc. of carbon tetrachloride. Yield=6.3 g.; M. P. 195–196°. Recrystallized in white needles from ethyl acetate; M. P. 200–201°.

## Method 2

To a finely divided mixture of 22 g. of o-aminophenol in 200 cc. of ethyl acetate was added 11 g. of cyanoacetylazide with stirring. The temperature of the mixture rose from 26–32°. It was evaporated to dryness and the tan residue 35 stirred with 200 cc. of water and filtered. The moist residue was transferred to a beaker containing a solution of 100 cc. of concentrated hydrochloric acid in 300 cc. of water. The mixture was stirred five minutes, filtered, washed on the funnel with water, and dried. Yield: 13 g.; M. P. 198–200°. The product was recrystallized in white needles from ethyl acetate; M. P. 200–201°.

## 5-CYANOACETAMINO-1-NAPHTHOL

A solution of 25 cc. of ethyl cyanoacetate and 5 cc. of quinoline was heated to 195° and 8 g. of 5-amino-1-naphthol added in small increments during 15 minutes while stirring. Heating was continued at 195–205° for one-half hour, alcohol being collected. The reaction mixture was cooled and poured into 150 cc. of ethyl ether. A small amount of gum was removed by filtration. The filtrate was treated with Darcō and filtered into 150 cc. of ligroin, the product being precipitated. 55 This solid was filtered and crystallized from

methanol and petroleum ether. Yield: 2.6 g.; M. P. 214-215°.

The aromatic amino developing agents used with the coupler compounds of our invention include the mono-, di- and tri-aminoaryl compounds and their derivatives formed by substitution in the amino group as well as in the ring such as alkylphenylenediamines and alkyltolylenediamines. These compounds are usually used in the salt form, such as the hydrochloride or the sulphate, which are more stable than the amines themselves. Suitable compounds are diethyl-p-phenylenediamine hydrochloride, monoethyl-p-phenylenediaminehydrochloride, dimethyl-p-phenylenediaminehydrochloride and dimethyl-p-phenylenediamine sulphate. Developing agents containing heterocyclic systems as described in U. S. Patent 2,196,739 are also suitable. The p-aminophenols and their substitution products may also be used where the amino group is unsubstituted. All of these compounds have an unsubstituted amino group which enables the oxidation products of the developer to couple with the color-forming compounds to form a dye image.

The following example illustrates a developing solution which may be used with the compounds of our invention.

|                                   |       |    |
|-----------------------------------|-------|----|
| A. p-Amino-diethylaniline sulfate | grams | 2  |
| Sodium sulfite (anhydrous)        | do    | 5  |
| Sodium carbonate (anhydrous)      | do    | 20 |
| Potassium bromide                 | do    | 2  |
| Water to 1 liter.                 |       |    |
| B. 2-cyanoacetaminophenol         | do    | 2  |
| Sodium hydroxide (2% solution)    | cc    | 50 |

For use, B is added to A.

Our development process may be employed for the production of colored photographic images in layers of gelatin or other carrier for the silver halide such as collodion, organic esters of cellulose or synthetic resins. The support for the emulsion may be a transparent material such as glass, cellulose ester or a non-transparent reflecting material such as paper or an opaque cellulose ester. The emulsion may be coated as a single layer on the support or as a superposed layer on one or both sides of the support. The superposed layer may be differentially sensitized to some natural color photographic images in the well-known manner.

The examples and compounds set forth in the present specification are illustrative only and it is to be understood that our invention is limited only by the scope of the appended claims.

We claim:

1. A color-forming photographic developer comprising a primary aromatic amino developing agent and a coupler compound having the formula:



where R is selected from the group consisting of aromatic nuclei of the benzene and naphthalene series and the position in the aromatic nucleus para to the hydroxyl group contains a substituent of the class consisting of hydrogen and a replaceable group.

2. A color-forming photographic developer comprising a primary aromatic amino developing agent and a coupler compound having the formula:



3. A color-forming photographic developer comprising a primary aromatic amino developing agent and a coupler compound having the formula:



3. A color-forming photographic developer comprising a primary aromatic amino developing agent and a coupler compound having the formula:



where R is selected from the group consisting of aromatic nuclei of the benzene and naphthalene series and the position in the aromatic nucleus para to the hydroxyl group contains a substituent of the class consisting of hydrogen and a replaceable group.

5. The method of producing a colored photographic image in a silver halide emulsion layer which comprises exposing said layer and developing it with a primary aromatic amino developing agent in the presence of a coupler compound having the formula:



where R is selected from the group consisting of aromatic nuclei of the benzene and naphthalene series and the position in the aromatic nucleus para to the hydroxyl group contains a substituent of the class consisting of hydrogen and a replaceable group.

8. A photographic emulsion for forming colored images comprising a silver halide emulsion having incorporated therein a coupler compound having the formula:



where R is selected from the group consisting of aromatic nuclei of the benzene and naphthalene series and the position in the aromatic nucleus para to the hydroxyl group contains a substituent of the class consisting of hydrogen and a replaceable group.

5

having incorporated therein a coupler compound having the formula:



ILMARI F. SALMINEN.  
ARNOLD WEISSBERGER.

#### REFERENCES CITED

The following references are of record in the file of this patent:

UNITED STATES PATENTS

| Number    | Name           | Date          |
|-----------|----------------|---------------|
| 2,108,602 | Mannes         | Feb. 15, 1938 |
| 2,441,491 | Kendall et al. | May 11, 1948  |

## FOREIGN PATENTS

10 Number Country Date  
576,891 Great Britain Apr. 25, 1946